

1

2,785,947

**PROCESS FOR PRODUCING DURABLE MECHANICAL EFFECTS ON CELLULOSE FABRICS BY APPLYING ACETALS AND PRODUCTS RESULTING THEREFROM**

Bernard H. Kress, Ambler, and Ellis Abrams, Philadelphia, Pa., assignors to Quaker Chemical Products Corporation, Conshohocken, Pa., a corporation of Pennsylvania

No Drawing. Application February 19, 1954.  
Serial No. 411,542

13 Claims. (Cl. 8—116)

This invention relates to the treatment of textile materials containing a substantial quantity of cellulose for the purpose of obtaining a variety of mechanical effects which are durable to laundering and dry cleaning.

This invention provides a new process for treating cellulosic textile materials in order to obtain such mechanical effects as can be obtained by various types of calendering. Glazed, embossed, Shreinered, chased, and moiré fabrics are among the types which can be produced by this new process. In general, the fabrics produced according to this invention are spot, soil, and crease resistant, stretch and shrink resistant, launderable by washing or dry cleaning, quick drying, ironable, and long wearing.

It is well-known in the art to obtain durable mechanical effects on cellulosic fabrics by impregnating same in aqueous solutions of thermosetting resins and acidic or potentially acidic catalysts. The impregnated fabrics are then dried at a relatively low temperature to a moisture content of about 10% and subsequently subjected to some type of hot calendering operation such as a glazer where the top roll travels more rapidly than the bottom roll. This operation glazes and partially sets the resin. Finally the fabric is passed through a curing oven operated at 300–400° F. for a period of about one-half to 5 minutes, the length of time varying inversely with the temperature of cure. Among the materials which have been recommended for this operation are urea-formaldehyde resins, thio-urea formaldehyde resins, melamine formaldehyde resins and various modified urea-formaldehyde resins.

All of the aforesaid materials which have been recommended as aids in "setting" the mechanical effects have several properties in common which differentiate them from the materials to be discussed in this invention. The materials hitherto known to the art are all thermosetting resin-forming products. When these materials are heated in an oven at 300° F. in presence of an acidic catalyst, they are converted to infusible products. Moreover, these materials are potential film formers. It has also been observed that these materials possess the unfortunate property of retaining chlorine to some degree when they are bleached with chlorine containing bleaches as might occur during home or commercial laundering operations. This factor limits the utility of fabrics treated with these materials by imposing conditions of special handling during laundering.

Another factor which imposes limitations on treatments with urea and melamine formaldehyde condensates is that many of these products emit objectionable odors during their application to textile materials and in certain cases these odors may persist in the finished fabric. In other instances objectionable odors may develop in the fabric after finishing. Furthermore, it has been observed that the degree of durability to laundering obtained through the use of these condensates is rather limited.

In view of the present state of the art, it is indeed un-

2

expected and surprising that durable washfast mechanical finishes can be obtained by treating textile fabrics with non-resin forming materials prior to calendering and curing.

5 An object of this invention is to obtain durable mechanical effects on cellulosic fabrics which will be free from the danger of chlorine retention due to bleaching. Incidental to these effects, we also aim to obtain fabrics which are resistant to spotting, soiling, and fraying and which possess improved crease resistance and substantial retention of tear and tensile strength.

A further object of this invention is to provide a treatment which will impart a minimum degree of discoloration to the treated fabric. Further, the treated material 15 will be free of objectionable odors or the disposition to form disagreeable odors. Moreover, the padding, drying, and curing operations will be substantially free of odors.

Further advantages of the invention will become apparent from the detailed description of the discovery 20 which follows.

It has been discovered that the above-mentioned objects may be accomplished by treating cellulosic textile materials, prior to drying, calendering, and curing, with non-volatile acetals of monoaldehydes and dialdehydes 25 containing up to eight carbon atoms in the presence of an acidic catalyst. The term "non-volatile" as applied here refers to non-volatility at the curing temperature of at least 250° F. In using the acetals according to this invention, at no time during the padding, drying, calendering, or curing operations is there a detectable odor of 30 acetals of formaldehyde.

Suitable aldehydes which may be converted to acetals in this process are formaldehyde, acetaldehyde, propanal, 35 butanal, glyoxal, and other mono- and dialdehydes containing not more than eight carbon atoms in the monomeric form, such as malonaldehyde, succinaldehyde, glutaraldehyde, adipaldehyde, hydroxyadipaldehyde, benzaldehyde, terephthalaldehyde, and the like.

40 Suitable alcohols which may be reacted with the above-mentioned aldehydes to form acetals are methanol, ethanol, propanol, isopropanol, butanol, methoxyethanol, ethoxyethanol, methoxyethoxyethanol, ethylene glycol, a propylene glycol, a butylene glycol, diethylene glycol, dipropylene glycol, dibutylene glycols and higher dialkyleneglycols, polyalkylene glycols, polyhydric alcohols such as glycerine, mannitol and sorbitol, and glycol monoethers and partial ethers of polyhydric alcohols.

45 In co-pending applications, Serial Numbers 403,078 filed January 8, 1954, and 403,057, filed January 8, 1954, we have disclosed individually that both monomeric acetals and polymeric acetals may be used in the presence of acidic catalysts for purposes of dimensional control of 50 cellulosic textile materials. We now find that these various acetals may be used to achieve the objects of this invention.

55 Suitable monomeric acetals applicable in this process are di-(hydroxyethoxyethyl) formal, di-(methoxyethoxyethyl) formal, di-(methoxyethyl) formal, di-(hydroxyethyl) acetal, glyoxal tetramethyl acetal, glyoxal tetraethyl acetal, glyoxal tetrabutyl acetal, 2-hydroxyadipaldehyde tetra-(methoxyethyl) acetal and mixed acetals such as 60 methyl methoxyethyl formal, malonaldehyde methyl triethyl acetal, glyoxal dibutyl dimethoxyethyl acetal, di-methoxymethoxyethyl ether, or methyl hydroxyethoxyethyl formal or mixtures thereof. In general, the acetals are prepared by reacting the aldehydes and alcohols in the presence of acidic catalysts by well-known procedures. Mixed acetals may be prepared by reacting the aldehyde 65 with a mixture of the alcohols or by carrying out an ex-

change reaction between a given acetal and the desired alcohol.

In general, our preferred monomeric acetals have boiling points above 125° C. and are derived from aldehydes containing one to eight carbon atoms and hydroxyl-bearing compounds containing at least one alkyl or alkylene radical, i. e. at least one continuous carbon chain possessing from one to six carbon atoms.

The polymeric acetals which are applicable in this invention are reaction products between an aldehyde and an alkylene or polyalkylene glycol. Typical polymeric acetals may be prepared from diethylene glycol and formaldehyde, ethylene glycol and formaldehyde, diethylene glycol, formaldehyde and glyoxal, diethylene glycol, sorbitol and formaldehyde, diethylene glycol and acetaldehyde, dipropylene glycol and hydroxyadipaldehyde and the like.

In general, those polymeric acetals which have proved useful in this invention may be made starting with ethylene glycol, a propylene glycol, a butylene glycol, dipropylene glycol, dibutylene glycols, and higher dialkylene glycols, polyalkylene glycols, mixtures thereof, or their mixtures with diethylene glycol which are reactive with formaldehyde or other aldehydes to form water soluble products or products which are dispersible in water, either alone or with the aid of appropriate adjuvants. Polyalkylene glycols, such as triethylene glycol, tetraethylene glycol, tripropylene glycol and the like may also be used, either alone or in admixture with the aforementioned glycols. Likewise polyols, such as glycerine, pentaerythritol and sorbitol, may be added to the alkylene glycols in amounts up to about 50 mole percent of the glycols for reaction with the aldehyde for forming water soluble or water dispersible products. Various materials, such as paraformaldehyde, formalin, trioxane, or methylal may be used as sources of formaldehyde. Other suitable aldehydes have been mentioned above and mixtures of these may be used in forming the condensation products. The term "alkylene" is understood to include a doubly unsatisfied aliphatic radical containing a substituted or unsubstituted straight chain possessing from two to four carbon atoms in the chain and having its unsatisfied valences on either adjacent or separated carbon atoms. If desired, the chains of the polymeric compounds may be terminated, either in whole or in part, by means of an alkyl radical possessing not more than eight carbon atoms.

Those of our acetals which are water soluble are applied to fabric with acidic catalysts from aqueous solutions. The water insoluble acetals were applied either from isopropanol solutions or from oil in water emulsions. In all cases, excellent retention of the mechanical deformation was obtained, no chlorine retention was observed and no obnoxious odors were noted during any of the processing steps.

The general application of these acetals involves padding cellulosic fabric through aqueous solutions or dispersions of the acetal containing from 2 to 25% by weight of the acetal. The padding bath must contain additionally some acidic-type catalyst, such as zinc chloride, maleic anhydride, oxalic acid, ammonium chloride, ammonium thiocyanate, citric acid, tartaric acid, phosphoric acid, ethyl acid phosphate, ammonium sulfate, sodium bisulfate, etc., in amount of about 5 to 200% by weight of the acetal content. Additionally, the bath may contain a lubricant or softener and various hand modifiers, such as polyvinyl alcohol, dextrin, starch, etc. The treated fabric may then be dried at an appropriate temperature to a moisture content of about 10 to 15% and then subjected to some suitable type of calendering at about 350 to 400° F. If a glazed chintz is desired, the two calender rolls will rotate at different speeds. Where an embossed effect is to be produced a pair of rolls is used, one in relief, the other in intaglio on the first. A Shreinered effect may be produced by calendering between one engraved and one plain roll. A linen-like effect may be produced by

chasing and a moiré effect can be obtained with specially engraved rolls. In any event, the calendering is carried out at elevated temperature and at pressures approximating 5 tons per square inch. Subsequent to the calendering operation, the fabric is cured at a temperature of at least 250° F. for about  $\frac{1}{2}$  to 10 minutes. The time of the cure varies inversely with the temperature. The cured fabric may then be washed lightly with a detergent and a mild alkali, rinsed thoroughly and dried.

The following illustrative examples will serve to explain our invention. Example I below illustrates the preparation of a typical polyformal as described in pending application, Serial Number 403,056 filed January 8, 1954.

*Example I*

|                   |       |       |
|-------------------|-------|-------|
| Diethylene glycol | moles | 1     |
| Paraformaldehyde  | do    | 1     |
| Sulfuric acid     | do    | 0.001 |
| 0 Toluene         | ml    | 25    |

The above components are mixed and heated under reflux in an apparatus equipped with a water trap. The solution is refluxed and water removed by azeotropic distillation. When 1 mole of water of reaction is removed the desired reaction is complete. The reaction mixture is neutralized with dilute sodium hydroxide solution and toluene is removed by evaporation in *vacuo* at temperatures not exceeding 110° C. The product is a viscous liquid, setting to a crystalline mass below 16° C. It is completely water soluble and also soluble in toluene and esters. The product has a molecular weight of 480 (Rast) and a hydroxyl equivalent of 220 which indicates it has a linear polymeric structure. It has a specific gravity of 1.155 at 94° F. The refractive index is  $N_D^{30}$ :1.462. The molecular weight and hydroxyl equivalent of the condensation product of this example indicate that this product possesses a polymeric structure, containing an average of four diethylene glycol units, as shown in the following formula:



where X and Y may be either H or  $-\text{CH}_2\text{OH}$ . Similarly, monofunctional alcohol modified condensation products may be prepared as in Example II.

### *Example II*

|                        | Parts |
|------------------------|-------|
| Diethylene glycol      | 101   |
| Beta methoxyethanol    | 4     |
| Paraformaldehyde (91%) | 30    |
| Toluene                | 20    |
| Sulfuric acid (99%)    | 0.1   |

The above materials were reacted as in Example I to yield a viscous liquid possessing a faint ethereal odor and soluble in water. Its polymeric nature was shown by Rast molecular weight determination which had a value of 637.

Similarly polyols may modify the polymeric condensation product.

### *Example III*

|                        | Parts |
|------------------------|-------|
| 5 Diethylene glycol    | 80    |
| Sorbitol-crystalline   | 32    |
| Paraformaldehyde (91%) | 30    |
| Toluene                | 20    |
| Sulfuric acid (99%)    | 1     |

These reactants were treated as in Example I. The product was a crystalline mass at room temperature, soluble in toluene and in water, and with virtually no odor.

The application of acetals is illustrated by the following examples.

## 5

## Example IV

An aqueous solution is prepared containing the following:

|                      | Percent |
|----------------------|---------|
| Product of Example I | 7.5     |
| Ammonium chloride    | 0.8     |

The solution was padded on 80 x 80 cotton sheeting at 100 percent pickup. The fabric was dried at 180° F. until it reached a moisture content of 11% and then calendered through heated rolls at 400° F. and under a pressure of about 5 tons per square inch. The fabric was then cured at 300° F. for 5 minutes and finally washed and dried. The fabric possessed a lustrous finish which was substantially retained even after soaping at the boil for 10 minutes. The crease resistance was substantially improved and the retention of tear and tensile strength was good. Chlorine retention tests conducted according to American Association of Textile Chemists and Colorists (A. A. T. C. C. 1952) tentative specification 69-52 showed no effects due to retained chlorine. A test with warm 5% sodium carbonate solution showed no indication of residual odor in the fabric.

## Example V

A solution containing the following materials was prepared:

|                       | Percent |
|-----------------------|---------|
| Dimethoxyethyl formal | 10      |
| Oxalic acid           | 1.0     |

Cotton sheeting (80 x 80) was treated as described in Example IV. The results were substantially the same as in Example IV.

## Example VI

An aqueous solution was prepared by dissolving the following materials:

|                      | Percent |
|----------------------|---------|
| Product of Example I | 7.5     |
| Zinc chloride        | 2.0     |

Cotton sheeting (80 x 80) was treated as in Example IV. The material possessed a soft hand and a deep lustrous appearance.

## Example VII

An aqueous solution containing the following materials was prepared:

|                                   | Percent |
|-----------------------------------|---------|
| Condensation product of Example I | 7.5     |
| Polyvinyl alcohol                 | 0.5     |
| Maleic anhydride                  | 0.5     |

Cotton sheeting (80 x 80) was treated as in Example IV. The treated fabric possessed a deep lustrous appearance and increased crispness over that shown in Example V.

## Example VIII

An aqueous impregnation bath was prepared containing the following materials:

|                                   | Percent |
|-----------------------------------|---------|
| Condensation product of Example I | 10.5    |
| Polyvinyl alcohol                 | 0.75    |
| Oxalic acid                       | 4.0     |

Light weight viscose rayon gabardine was padded through the solution at 70% pick up at 7 tons roll pressure. The fabric was carefully dried until approximately 10% excess moisture was left on the cloth. The fabric was then embossed at about 350° F. and approximately 5 tons per square inch pressure.

The embossed cloth was then passed through a curing oven at 340° F. at 20 yds./min. and neutralized and framed. The embossed pattern showed good retention on laundering.

## 6

## Example IX

|                                   | Pounds |
|-----------------------------------|--------|
| Condensation product of Example I | 165    |
| Polyvinyl alcohol                 | 7.5    |
| Ammonium chloride                 | 17.0   |
| Water to make 180 gallons.        |        |

5 Cotton sheeting 38", 80/96, 4.85 yds./lb. was impregnated with the above solution and squeezed until a 75% pick up of solution was obtained based on the weight of the fabric. The fabric was then dried on cans maintained at 200° F. at 75 yds./min. and framed at 36 1/4". The fabric was then Shreinered and cured at 22 yds./min. at 330° F., and finally neutralized continuously and framed at 36 1/4". The fabric was then calendered to increase the luster. This fabric showed good luster retention through repeated laundering and possessed a marked degree of soil and crease resistance.

## Example X

|                                  | Percent |
|----------------------------------|---------|
| Glyoxal tetramethoxyethyl acetal | 10      |
| Oxalic acid                      | 1       |
| Water                            | 85      |

20 The acetal was prepared according to directions given in U. S. Patent 2,321,094. The solution was used to impregnate 80 x 80 cotton sheeting as described in Example IV. A durably glazed fabric was obtained.

## Example XI

The following solution was prepared:

|                                  | Percent |
|----------------------------------|---------|
| Glyoxal tetramethoxyethyl acetal | 10      |
| Oxalic acid                      | 1.5     |
| Water                            | 86.5    |

This solution was applied to 80 x 80 cotton sheeting as in Example IV with similar results.

## Example XII

|                       | Percent |
|-----------------------|---------|
| Product of Example II | 7.5     |
| Polyvinyl alcohol     | 0.5     |
| Zinc chloride         | 2.0     |
| Water                 | 90.0    |

40 This solution was used to impregnate cotton sheeting (80 x 96) as described in Example IV. The fabric was dried on a tenter frame to a moisture content of 11.5% and passed through specially engraved calender rolls at 375° F. to produce a moiré effect. The fabric was then cured at 400° F. for 30 seconds, washed and dried. The pattern retention on repeated laundering was excellent. No objectionable odors were noticed during the operations and the fabric showed no effects due to chlorine retention.

## Example XIII

60 The following solution was applied to cotton sheeting 80 x 80 as described in Example XII and with similar results:

|                        | Percent |
|------------------------|---------|
| Product of Example III | 8.0     |
| Oxalic acid            | 0.8     |
| Water                  | 89.0    |

70 The term "cellulose textile material" is intended to include fabrics, whether knitted, woven or felted, consisting of natural cellulose, regenerated cellulose, such as viscose rayon, cuprammonium rayon, and hydrolyzed cellulose acetate and mixtures thereof. Also included are fabric blends containing a preponderance of cellulosic type components.

The invention herein described is useful in a wide range 75 of mechanical finishing operations. While we have de-

scribed several of these procedures, our invention is not limited thereto but is applicable to any operation wherein it is desired to cause a mechanical surface deformation of a textile material to become durable to laundering. In the appended claims, therefore, we do not intend to restrict ourselves to the specific methods and conditions given above as illustrative; by the term physically modifying therein employed we mean that result of modification of the surface of a textile material by any appropriate mechanical means and under any suitable conditions of time, temperature, and pressure to impart to the surface a distinctive appearance, such as moiré, wave, crepe, stamping, lucid gloss, matted gloss, silk lustre, imitation mercerizing and various other surface effects and designs.

We claim:

1. The process of modifying the surface appearance of a cellulose textile material which comprises applying to a cellulose textile material an aqueous bath containing an acidic catalyst and an acetal of an aldehyde selected from the group consisting of aliphatic and carbocyclic aldehydes having 1 to 8 carbon atoms in monomeric form and mixtures of the aforesaid aldehydes, and an aliphatic hydroxyl-bearing compound selected from the group consisting of aliphatic monohydric alcohols containing from 1 to 5 carbon atoms, monoalkylene and polyalkylene glycols in which the alkylene radical has from 2 to 4 carbon atoms in a straight chain, and aliphatic polyhydric alcohols containing from 3 to 6 hydroxyl groups and from 3 to 6 carbon atoms and mixtures of the aforesaid aliphatic hydroxyl-bearing compounds, said acetal having a boiling point above about 125° C., said catalyst being present in amount from about 5% to about 200% by weight of the acetal content in said bath and said acetal being present in amount from about 2% to about 25% by weight of the bath, modifying the surface appearance of the treated textile material by applying pressure thereto and heating the textile material at an elevated temperature until the cellulose and acetal react and the surface appearance of the textile material is modified and stabilized to laundering.

2. The process of modifying the surface appearance of a cellulose textile material which comprises applying to a cellulose textile material an aqueous bath containing an acidic catalyst and an acetal of an aldehyde selected from the group consisting of aliphatic and carbocyclic aldehydes having 1 to 8 carbon atoms in monomeric form and mixtures of the aforesaid aldehydes, and an aliphatic hydroxyl-bearing compound selected from the group consisting of aliphatic monohydric alcohols containing from 1 to 5 carbon atoms, monoalkylene and polyalkylene glycols in which the alkylene radical has from 2 to 4 carbon atoms in a straight chain, and aliphatic polyhydric alcohols containing from 3 to 6 hydroxyl groups and from 3 to 6 carbon atoms and mixtures of the aforesaid aliphatic hydroxyl-bearing compounds, said acetal having a boiling point above about 125° C., said catalyst being present in amount from about 5% to about 200% by weight of the acetal content in said bath and said acetal being present in amount from about 2% to about 25% by weight of the

bath, modifying the surface appearance of the treated textile material by applying pressure thereto and heating the textile material at a temperature of at least about 250° F. for about 1/2 to 10 minutes until the cellulose and acetal react and the surface appearance of the textile material is modified and stabilized to laundering.

3. The process of modifying the surface appearance of a cellulose textile material as defined in claim 1 wherein the bath contains an acetal of diethylene glycol and formaldehyde.

4. The process of modifying the surface appearance of a cellulose textile material as defined in claim 1 wherein the acetal in the aqueous bath is the condensation product of diethylene glycol, sorbitol and formaldehyde.

5. The process of modifying the surface appearance of a cellulose textile material as defined in claim 1 wherein the acetal in the aqueous bath is di-(methoxyethyl) formal.

6. The process of modifying the surface appearance of a cellulose textile material as defined in claim 1 wherein the acetal in the aqueous bath is malonaldehyde methyl triethyl acetal.

7. The process of modifying the surface appearance of a cellulose textile material as defined in claim 1 wherein the acetal in the aqueous bath is glyoxal tetra-(methoxyethyl) acetal.

8. Cellulose textile material having a durable surface appearance resisting laundering made by the process of claim 1.

9. Cellulose textile material having a durable surface appearance resisting laundering made by the process of claim 3.

10. Cellulose textile material having a durable surface appearance resisting laundering made by the process of claim 4.

11. Cellulose textile material having a durable surface appearance resisting laundering made by the process of claim 5.

12. Cellulose textile material having a durable surface appearance resisting laundering made by the process of claim 6.

13. Cellulose textile material having a durable surface appearance resisting laundering made by the process of claim 7.

#### References Cited in the file of this patent

##### UNITED STATES PATENTS

2,207,740 Kaase et al. ----- July 16, 1940  
2,350,350 Gresham ----- June 6, 1944  
2,360,477 Dahle ----- Oct. 17, 1944

##### FOREIGN PATENTS

291,473 Great Britain ----- June 1, 1928  
527,888 Great Britain ----- Oct. 17, 1940  
547,846 Great Britain ----- Sept. 15, 1942

##### OTHER REFERENCES

Marsh, John T.: An Introduction to Textile Finishing, 1948, p. 381.